# EUROPEAN PATENT APPLICATION

(11) **EP 0 896 252 A1**
(43) Date of publication of application: **10.02.1999**
(21) Application number: 98114571.7
(22) Date of filing: 03.08.1998
(51) Int. Cl.: G03G 9/08

(54) **Toner for developing latent electrostatic images and image formation method using the toner**

(30) Priority: 04.08.1997 JP 221225/97; 31.07.1998 JP 229492/98
(71) Applicant: Ricoh Company, Ltd., Tokyo 143-8555 (JP)
(72) Inventor: Sugimoto, Shohichi, Ohta-ku, Tokyo, 143-8555 (JP); Kuramoto, Shinichi, Ohta-ku, Tokyo, 143-8555 (JP)
(74) Representative: Barz, Peter, Dr.

(57) **Abstract**

A toner for developing latent electrostatic images to toner images for use in an intermediate transfer image formation method is proposed, which is composed of toner particles including a coloring agent and a binder resin, with an average particle size in a range of 5 to 10 µm and an aggregation degree of 5 to 20%, and a method of producing the toner, and an intermediate transfer image formation method using the toner are proposed.

## Description

The present invention relates to a toner for developing latent electrostatic images to toner images for use in an intermediate transfer image formation method comprising the steps of forming a thin layer of toner on a toner bearing member, triboelectrically charging the toner to a predetermined polarity using a triboelectric charging member, developing latent electrostatic images formed on an image bearing member to toner images with the toner, transferring the developed toner images to an intermediate image transfer member, such as an endless-belt-shaped intermediate image transfer member, thereby performing a first image transfer, and transferring the toner images transferred by the first image transfer from the intermediate image transfer member to an image transfer material, thereby performing a second image transfer. The present invention also relates to a method of producing the above-mentioned toner, and also relates to the above-mentioned intermediate transfer image formation method.

There is known an intermediate transfer image formation method by which a plurality of visible developed color images is successively formed on an image bearing member such as a photoconductor and is then transferred in a superimposed manner to an intermediate member which runs along an endless path, such as an endless-belt-shaped intermediate image transfer member, thereby performing a first image transfer, and the thus transferred images are then transferred to an image transfer material, thereby performing a second image transfer,

Such an intermediate transfer image formation method is particularly used in an image formation method using an image transfer method of superimposing black, cyan, magenta and yellow toner images in a full-color image formation apparatus which subjects an original image subjected to color separation and then reproduces the original image, using subtractive mixtures of toners such as black, cyan, magenta and yellow toners.

In such an image formation method as mentioned above, it may occur that in a final image bearing material such as an image transfer sheet, images with non-image transferred spots are formed due to the occurrence of local non-image transfer in the course of the steps of the above-mentioned first and second image transfers. If such non-image transferred spots are formed in solid images, the images are worm-eaten like images with non-image transferred spots having certain areas, and if such non-image transferred spots are formed in line images, broken line images are formed. In order to prevent the formation of such abnormal images, it is important to improve the image transfer technology. Under such circumstances, the following improved image transfer technologies have been proposed:

### 1. Reduction of image transfer nip pressure (Technology 1):

In this technology, as disclosed in Japanese Laid-Open Patent Applications 1-177063 and 4-284479, a nip pressure between a photoconductor and an intermediate image transfer member is set at an appropriate value so as to improve image transfer performance and to prevent the formation of images with worm-eaten-like non-image transferred spots.

For instance, in the case where the first image transfer is conducted from the photoconductor to the intermediate image transfer member, when the first image transfer is carried out, the photocoductor and the intermediate image transfer member are in pressure contact with each other by mechanical force or electrostatic force with an image transfer nip pressure, so that pressure is applied to the toner which is present between the photoconductor and the intermediate image transfer member. The Van der Waals forces between the molecules of the toner are increased as the distance theretween is decreased by the pressure applied thereto, and the attraction between the molecules of the toner is also increased by the aggregation of the toner. For these reasons, this technology indicates that it is preferable that the nip pressure be decreased in order to obviate the formation of the worm-eaten-like transferred images.

### 2. Reduction of the surface energy of the intermediate image transfer member (Technology 2):

2-1 The wettability of the intermediate image transfer member is set at an increased specific value, whereby the image transfer performance is improved and the formation of worm-eaten-like transferred images is obviated.
   In this technology, which is disclosed in Japanese Laid-Open Patent Applications 2-198476 and 2-212867, an intermediate image transfer member with small wettability, that is, with small surface energy, is used in an attempt to prevent the formation of worm-eaten-like transferred images.
2-2 A multi-layered intermediate image transfer member with an exterior layer having excellent releasability is used, whereby the image transfer performance is improved and the formation of worm-eaten-like transferred images is obviated. This technology is disclosed in Japanese Laid-Open Patent Applications 62-293270, 6-204255, 5-204257 and 5-303293.
2-3 A material having excellent releasability is supplied to the surface of an intermediate image transfer member, whereby the image transfer performance is improved and the formation of worm-eaten-like transferred images is obviated. This technology is disclosed in Japanese Laid-Open Patent Application 58-187968.
   In this technology, the surface tension of the intermediate image transfer member is reduced, and the releasability of the intermediate image transfer member away from toner is improved, whereby the image transfer performance of toner images to the image transfer member is improved. Generally, the adhesion between different materials is represented by a function of the surface tensions thereof, so that as the surface tension of the intermediate image transfer member is increased, the adhesion of the intermediate image transfer member to the toner is also increased as conventionally known. In the case of a pure material, the surface tension thereof is synonymous with the surface energy thereof. Even in the case of a composite material, the surface tension thereof and the surface energy thereof are generally used interchangeably to indicate a representative characteristic of the material as in the case of the wettability thereor.

### 3. Removal of toner filming layer from the surface of the intermediate image transfer member (Technology 3):

In this technology, the surface of the intermediate image transfer member is subjected to filming polishing, thereby the formation of worm-eaten-like transferred images with time is prevented, while the image transfer performance thereof is maintained. This technology is proposed in Japanese Laid-Open Patent Applications 5-273893, 5-307344, 5-313526 and 5-323802.

In the above-mentioned Technologies 1 to 3, if the objects of Technology 2 are accomplished so that the surface tension of the intermediate image transfer member is reduced as desired, no toner filing layer is formed and accordingly Technology 3 will become unnecessary. In other words, Technology 3 is a supplement to Technology 2.

Prior art for preventing the formation of worm-eaten-like transferred images at the second image transfer is as follows;

When a roller is used for roller image transfer in the second image transfer, worm-eaten-like transferred images are apt to be formed for the following two reasons A and B:
A. When full-color images are formed, a toner layer becomes thick in the course of the formation of full-color images, and strong adhesion force, that is, non-Coulomb force, is mechanically generated between (a) the surface of the intermediate image transfer member and (b) the toner by the contact pressure of the roller applied to the toner, so that the substantial density of the toner is increased, and the Van der Waals force is also increased since toner particles mutually come close to each other. The result is that the adhesion of the toner particles in the toner is increased.
B. In the course of the repetition of image formation process, a so-called toner filming phenomenon (i.e. a phenomenon of depositing toner in the shape of a thin film on the surface of the intermediate image transfer member) takes place, so that adhesive force is generated between the toner and the surface of the intermediate image transfer member. Generally, as the material for the intermediate image transfer member, a material with small surface tension or small surface energy is selected in order to avoid the occurrence of the toner filming phenomenon. Even when such a selection is made, adhesive force (i), which corresponds to the surface tension between the intermediate image transfer medium and the toner, is inevitably generated, and once the toner filming phenomenon takes place, the adhesive force (i) between the intermediate image transfer medium and the toner depends upon such an adhesive force (ii) that is determined by the surface tension of the toner particles of the toner. The adhesive force (ii) is obviously greater than the adhesive force (i). Thus, the adhesive force between the toner particles of the toner is increased, so that images with worm-eaten-like non-image transferred spots are formed.

A technology for avoiding the formation of the above-mentioned non-image transferred spots in the images is proposed in U.S. Patent No. 5,053,827 (METHOD AND APPARATUS FOR INTERMITTENT CONDITIONING OF A TRANSFER BELT).

In the technology disclosed in this U.S. Patent, a roller composed of a fluorine-containing material having a smaller surface energy than that of an intermediate image transfer belt serving as the intermediate image transfer member is brought into contact with the surface of the intermediate image transfer belt, as conditioning means for reducing the surface energy of the intermediate image transfer belt, thereby performing a conditioning process for reducing the surface energy of the intermediate image transfer belt. Further, it is disclosed that an intermediate image transfer belt composed of polycarbonate is used.

The inventors of the Present invention conducted image transfer tests, using an image formation apparatus using a one-component type developer as shown in Figure.

In a first image transfer test, as the intermediate image transfer belt, an intermediate image transfer belt made of polycarbonate resin was employed. The result was that in the course of repeated image formation and transfer with time, worm-eaten-like transferred images are formed at the second image transfer.

In a second image transfer test, the above-mentioned first test was repeated in the same manner as mentioned above except that an appropriate amount of zinc stearate was applied to the surface of the above intermediate image transfer belt as a lubricant. The result was that the formation of worm-eaten-like transferred images at the second image transfer was successfully prevented, but blurred images were formed. It was discovered that the formation of the blurred images was caused by the reduction of the deposited amount of the toner on the intermediate image transfer belt at the first image transfer.

In a third image transfer test, the above-mentioned first test was repeated in the same manner as mentioned above except that as the intermediate image transfer belt, an intermediate image transfer belt made of ethylene-tetrafluoroethylene copolymer (ETFE) was employed. The result was that blurred images were formed from an initial stage of the image transfer.

These three tests can be compared with the above-mentioned conventional example shown in U.S. Patent No. 5,053,827 as follows:

In the above-mentioned conventional example, the surface energy of the intermediate image transfer belt is controlled to be set at a certain level by the conditioning process, while in the above-mentioned tests, although the surface of the photoconductor serving as a toner bearing member is polished, for example, by a cleaning brush roller, toner is deposited in the form of a thin film on the surface thereof with time in the same manner as with the case of the intermediate image transfer belt, or the surface of the photoconductor is smeared with charged gases such as ozone and NOx which are generated by corona charging in the course of the repeated image formation and transfer, so that the surface energy of the surface of the photoconductor is gradually increased with time. The result is that toner is apt to be mechanically deposited on the Surface of the photocoductor and eventually the image transfer performance of the photoconductor is considered to be impaired with time.

The above-mentioned impairment of the image transfer performance will bring about not only the above-mentioned imperfect image transfer with the formation of non-transferred spots in the images, but also the transfer of black toner images developed with a single black toner back to the surface of the photoconductor in such an image formation apparatus that forms toner images by successively superimposing black, cyan, magenta and yellow toners in this order.

Furthermore, as mentioned in the above third image transfer test, when the intermediate image transfer belt made of ETFE was used, blurred images were formed from an initial stage of the image transfer. It is considered that this was because the difference between the surface energy Of the photoconductor and the surface energy of the intermediate image transfer belt was already large at the initial stage of the image transfer.

In order to avoid these problems, in the above-mentioned U.S. Patent, when the surface energy of the intermediate image transfer belt becomes excessively large, the conditioning process is performed. Specifically, when the number of copies made exceeds a preset number of copies, the conditioning process is performed.

The above image transfer method, however, has a potential problem that developed images are dull, unclear and, particularly unsharp in line images, and are not in the right positions, which is collectively hereinafter referred to as dull image formation.

In order to improve the image quality obtained by the above-mentioned image transfer method, the following methods have been conventionally proposed:
(1) Toner images made of a toner with high resistivity are non-electrostatically transferred to an intermediate image transfer medium, and the thus transferred toner images are then transferred via a recording sheet with the application of pressure, using a heat application roller as disclosed in Japanese Laid-open Patent Application 63-34570.
(2) Toner images made of an electroconductive toner are non-electrostatically transferred to an intermediate image transfer medium, and the thus transferred toner images are then transferred via a recording sheet with the application of pressure, using a heat application roller as disclosed in Japanese Laid-Open Patent Application 63-34571.
(3) Whenever toner images are transferred to an intermediate image transfer sheet, the transferred toner images are electrically quenched, using a sheet separation charger as disclosed in Japanese Laid-open Patent Application 1-282571.
(4) The image transfer potential at a final image transfer stage is set larger than that at an image transfer stage immediately before the final image transfer stage, and a predetermined voltage is applied to an intermediate image transfer medium between each image transfer step as disclosed in Japanese Laid-Open Patent Application 2-183276.
(5) Means for quenching electric charges on an intermediate image transfer medium is provided at a predetermined position on a path which leads to means for transferring visible images to a transfer sheet from the intermediate image transfer medium as disclosed in Japanese Laid-Open Patent Application 4-147170.

However, in the above-mentioned methods (1) and (2), the recording sheet is required to perform the image transfer with the application of heat and pressure by the heating roller is required.

Further, in the above-mentioned methods (3) to (5), the quenching means and voltage application means and/or control means therefor are required, so that the mechanical control of such means involves complicated steps and it is not easy to make compact in size the image formation apparatus therefor.

In Japanese Laid-Open Patent Applications 7-181732 and 7-161733, it is described that the toner particles of the toner for use in the image formation apparatus or the intermediate image transfer type are made spherical in shape to eliminate the problems of non-transfer of the images and the scattering of the toner during the image transfer step. The image transfer performance is not sufficiently improved by the method proposed in these prior art for use in practice, and the problem of the toner scattering is not substantially solved by the method disclosed in these references. In particular, in a mono-component development, by use of the toner comprising the spherical toner particles, the triboelectric charging of the toner particles by a blade becomes insufficient, so that the charging of the toner becomes unstable.

It is therefore a first object of the present invention to provide a toner for developing latent electrostatic images to toner images, without the formation of worm-eaten-like images with non-transferred spots, thicker images than original images, deposition of the toner on the background of the images, which is used in an intermediate transfer image formation method comprising the steps of forming a thin layer of toner on a toner bearing member, triboelectrically charging the toner to a predetermined polarity using a triboelectric charging member, developing latent electrostatic images formed on an image bearing member to toner images with the toner, transferring the developed toner images to an intermediate image transfer member which runs along an endless path, thereby subjecting the developed toner images to a first image transfer, and transferring the toner images transferred to the intermediate image transfer member to an image transfer material, thereby subjecting the developed toner images to a second image transfer.

A second object of the present invention is to provide a method of producing the above toner.

A third object of the present invention is to provide an intermediate transfer image formation method, using the above-mentioned toner.

The first object of the present invention can be achieved by a toner which comprises toner particles comprising a coloring agent and a binder resin, with an average particle size in a range of 5 to 10 µm and an aggregation degree of 5 to 20%, preferably 7 to 15%, more preferably 9 to 12%.

The toner or the present invention may further comprise finely-divided particles of silica which are made hydrophobic in an amount ratio of 0.1 to 1.0 parts by weight to 100 parts by weight of the toner.

The toner of the present invention may further comprise finely-divided particles of titanium oxide in an amount ratio of 0.1 to 1.2 parts by weight to 100 parts by weight of the toner.

The toner of the present invention may further comprise both (a) finely-divided particles of silica which are made hydrophobic and (b) finely-divided particles of titanium oxide in a parts-by-weight ratio of 1 : 9 to 6 : 4.

It is preferable that the binder resin for the toner particles of the toner of the present invention be a polyol resin.

The second object of the present invention can be achieved by a method comprising the steps of:
stirring toner particles comprising a coloring agent and a binder resin alone, and then
mixing the toner particles with an at least one additive component.

In the above method of the present invention, the additive component may be selected from the group consisting of (a) finely-divided particles of silica which are made hydrophobic and (b) finely-divided particles of titanium oxide

The third object of the present invention can be achieved by an intermediate transfer image formation method which comprises the steps of:
forming a thin layer of toner on a toner bearing member, triboelectrically charging the toner to a predetermined polarity using a triboelectric charging member, developing latent electrostatic images formed on an image bearing member to toner images with the toner, transferring the developed toner images to an intermediate image transfer member which runs along an endless path, thereby subjecting the developed toner images to a first image transfer, and transferring the toner images transferred to the intermediate image transfer member to an image transfer material, thereby subjecting the developed toner images to a second image transfer, wherein as the toner is used a toner which comprises toner particles comprising a coloring agent and a binder resin, with an average particle size in a range of 5 to 10 µm and an aggregation degree of 5 to 20%.

In the above-mentioned intermediate transfer image formation method of the present invention, the toner may further comprise finely-divided particles of silica which are made hydrophobic in an amount ratio of 0.1 to 1.0 parts by weight to 100 parts by weight of the toner.

Furthermore, in the above-mentioned intermediate transfer image formation method of the present invention, the toner may further comprise finely-divided particles of titanium oxide in an amount ratio of 0.1 to 1.2 parts by weight to 100 parts by weight of the toner.

Furthermore, in the above-mentioned intermediate transfer image formation method of the present invention, the toner may further comprise (a) finely-divided particles of silica which are made hydrophobic and (b) finely-divided particles of titanium oxide in a parts-by-weight ratio of 1: 9 to 6 : 4.

In the above-mentioned intermediate transfer image formation method, it is preferable that the binder resin for use in the toner particles be a polyol resin.

A more complete appreciation of the invention and many of the attendant advantages thereof will be readily obtained as the same becomes better understood by reference to the following detailed description when considered in connection with the accompanying drawing, wherein:

Figure shows a schematic cross-sectional view of a one-component type development apparatus for use in the present invention

The toner of the present invention comprises toner particles comprising a coloring agent and a binder resin, with an average particle size in a range of 5 to 10 µm and an aggregation degree of 5 to 20%, preferably 7 to 15%, more preferably 9 to 12%.

When the average particle size of the toner is larger than the above-mentioned average particle size, sharp images cannot be obtained, while when the average particle size of the toner is smaller than the above-mentioned average particle size, the fluidity of the toner is extremely reduced so that images with non-transferred spots are formed during the image transfer step.

The aggregation degree of the toner is widely used as a characteristic which indicates the fluidity of the toner. The higher the spherical degree of the toner particles, the smaller the aggregation degree, and the higher the fluidity of the toner.

Generally, in a two-component type development method, toner is treated so as to make the toner particles thereof spherical to improve the fluidity of the toner and to reduce the occurrence of non-transferred stops in toner images. However, as mentioned above, in a mono-component type development method, when the toner is treated so as to make the toner particles spherical, the triboelectric charging of the toner particles in contact with a triboelectric charging member becomes insufficient, so that the charging of the toner becomes unstable and images obtained are poor in quality.

When the fluidity of the toner is excessively low, worm-eaten-like and unsharp images are formed.

In sharp contrast to this, in the present invention, by setting the aggregation degree of the toner in the range of 5 to 20%, the formation of worm-eaten-like images with non-transferred spots, thicker images than the original images, and the deposition of the toner on the background of the images can be prevented at the same time.

The aggregation degree is determined as follows:

On a 22 µm mesh sieve is placed a 45 µm mesh sieve, and a 75 µm mash sieve is then placed on the 45 µm mesh sieve, so that the 75 µm mesh sieve serves as an uppermost sieve. In this 75 µm mesh uppermost sieve is placed 2 g of a toner sample, and the toner sample in the uppermost sieve is vibrated for 30 seconds, using a commercially available powder tester (made by Hosokawa Micron Corporation), and the amount of the toner sample remaining in each of the three sieves is measured. The aggregation degree is calculated from the following formula:$\text{Aggregation degree (%) = {(the remaining amount of the toner sample in the 75 µm mesh sieve) + 0.6 x (the remaining amount or the toner sample in the 45 µm mesh sieve) + 0.2 x (the remaining amount of the toner sample in the 22 µm mesh sieve)} /2.0 x 100}$

The aggregation degree of the toner can be adjusted by changing the shape and/or the particle size distribution of the toner particles of the toner, or by replacing the kind of an additive to be added to the toner and changing the amount of the additive added. As mentioned above, it is not always suitable for the present invention to make the toner particles spherical in shape in order to adjust the aggregation degree.

With respect to the particle size distribution of the toner particles, when the average particle size of the toner particles is excessively small, the amount of an additive to be externally added to the toner has to be increased to secure the necessary fluidity of the toner. This is not suitable for the present invention. On the other hand, when the average particle size of the toner particles is excessively large, a problem that the resolution of the toner when producing line images is significantly reduced, Generally, there is a tendency that when the amount of an additive to be added to the toner is increased, the aggregation degree of the toner is decreased, while when the amount of the additive is decreased, the aggregation degree of the toner is increased.

Examples of the additive for use in the toner of the present invention are finely-divided particles of silica which are made phydrophobic, and finely-divided particles of titanium oxide. It is preferable that finely-divided particles of silica which are made phydrophobic, and finely-divided particles of titanium oxide be used in combination, particularly for gaining more freedom when avoiding the above-mentioned potential problem that developed images are dull, unclear and, particularly unsharp in line images, and are not in the right positions, although the reasons therefor are unknown.

Specific examples of the finely-divided particles of silica which are made hydrophobic are "HDK H 2000", "HDK H 2000/4", "HDK H 2050EP", and "HVK21" (Trademark) made by Hoechst Japan Limited; "R972", "R974", "RX200", "RY200", "R202", "R805", and "R812" (Trademark) made by Nippon Aerosil Co., Ltd.; and "TS720" (Trademark) made by Cabot Corporation.

Specific examples of the finely-divided particles of titanium oxide are "P-25" (Trademark) made by Nippon Aerosil Co., Ltd.; "STT-30" and "STT-65C-S" (Trademark) made by Titan Kogyo K.K.; "TAF-140" (Trademark) made by Fuji Titanium Industry Co., Ltd.; "MT-150W", "MT-500B" and "MT-600B" (Trademark) made by Tayca Co., Ltd.

Finely-divided particles of titanium oxide which are treated so as to be hydrophobic can also be employed. Examples of such hydrophobically treated finely-divided particles of titanium oxide are anatase-type crystalline, rutile-type crystalline, and amorphous. Specific examples of such hydrophobically treated finely-divided particles of titanium oxide are "TS-805" (Trademark) made by Nippon Aerosil Co., Ltd. "MT-100S", "MT-100T", "MT150A" and "MT150AFM" (Trademark) made by Tayca Co., Ltd.; "STT-30A" and "STT-62S-S" (Trademark) made by Titan Kogyo K.K.; "MT-100S" and "MT-100T" (Trademark) made by Tayca Co., LTd.; "IT-5" (Trademark) made by Ishihara Sangyo Kaisha, Ltd.

The hydrophobically treated finely-divided particles of silica, titania and alumina can be obtained by treating hydrophilic finely-divided particles of silica, titania and alumina respectively to a silane coupling agent such as methyltrimethoxy silane, methyltriethoxy silane, or octyltrimethoxy silane, or by subjecting hydrophilic finely-divided particles of silica, titania and alumina to a polysiloxane treatment.

It is preferable that the toner of the present invention further comprise finely-divided particles of silica which are made hydrophobic in an amount ratio of 0.1 to 1.0 parts by weight to 100 parts by weight of the toner, more preferably in an amount ratio of 0.2 to 0.8 parts by weight to 100 parts by weight of the toner. When the amount of the finely-divided particles of the silica is more than 1.0 part by weight to 100 parts by weight of the toner, the above-mentioned potential problem that developed images are dull, unclear and, particularly unsharp in line images, and are not in the right positions tends to occur, while when the amount of the finely-divided particles of the silica is less than 0.1 parts by weight to 100 parts by weight of the toner, the aggregation degree of the toner excessively increases, so that images with non-transferred spots tend to be formed.

It is also preferable that the toner of the present invention further comprise finely-divided particles of titanium oxide in an amount ratio of 0.1 to 1.2 parts by weight to 100 parts by weight of the toner, more preferably in an amount ratio of 0.3 to 1.0 parts by weight to 100 parts by weight of the toner.

It is also preferable that the toner of the present invention further comprise both (a) the above-mentioned finely-divided particles of silica which are made hydrophobic and (b) the above-mentioned finely-divided particles of titanium oxide in a parts-by-weight ratio of 1 : 9 to 6 : 4, more preferably in a parts-by-weight ratio of 2 : 8 to 5: 5, furthermore preferably in a parts-by-weight ratio of 3 : 7 to 5: 5.

When producing a toner of the present invention, which comprises toner particles comprising a coloring agent and a binder resin, and at least one additive component, it is preferable that the toner particles be stirred first alone and then the additive component be mixed with the toner particles in order to prepare a toner which has the above-mentioned effects for use in the intermediate image transfer method. Although the reasons why the above-mentioned is effective for obtaining the above-mentioned effects is unknown, it is considered that this is because edges of toner particles are appropriately removed without causing side effects of lowering the charging performance of the toner, whereby, for instance, the formation of images with non-transferred spots is prevented.

It is also preferable that the toner particles be stirred first alone immediately before the additive component is mixed with the toner particles, more specifically about 5 minutes before the mixing of the additive component with the toner particles. It is also preferable that the above mixture be stirred for 200 to 400 seconds, whereby even if a plurality of additive components is mixed with the toner particles, uniform mixing can be performed.

In addition, the toner of the present invention may further comprise additives, for example, fatty acid metallic salts such as zinc stearate and aluminum stearate, metallic oxides such as aluminum oxide, tin oxide and antimony oxide, and fluoropolymers.

As other components for use in the toner of the present invention, any and all conventionally known materials can be employed.

Specific examples of such a binder resin for use in the present invention include homopolymers of styrene or substituted styrenes such as polystyrene, poly-p-chlorostyrene copolymer, and polyvinyltoluene; styrene copolymers such as styrene - p-chlorostyrene copolymer, styrene - propylene copolymer, styrene - vinyltoluene copolymer, styrene - vinylnaphthalene copolymer, styrene - methyl acrylate copolymer, styrene - ethyl acrylate copolymer, styrene - butyl acrylate copolymer, styrene - octyl acrylate copolymer, styrene - methyl methacrylate copolymer, styrene - ethyl methacrylate copolymer, styrene - butyl methacrylate copolymer, styrene - methyl α-chloro-methacrylate copolymer, styrene acrylonitrile copolymer, styrene - vinyl methyl ketone copolymer, styrene - butadiene copolymer, styrene - isoprene copolymer, styrene - acrylonitrile - indene copolymer, styrene - maleic acid copolymer, and styrene - maleic acid ester copolymer; polymethyl methacrylate; polybutyl methacrylate; polyvinyl chloride; polyvinyl acetate; polyethylene; polypropylene; polyester; epoxy resin; epoxy polyol resin?; polyurethane; polyvinyl butyral; polyacrylic resin; rosin; modified rosin; terpene resin; aliphatic or aliphatic hydrocarbon resin; aromatic petroleum resin; chlorinated paraffin; and paraffin wax.

Non-compatible combinations of resins can be employed, for example, combinations of resins of which characteristics are largely different, such as combinations of styrene-butyl acrylate copolymer and polyester, styrene-butyl acrylate copolymer and epoxy resin, and styrene-butyl acrylate copolymer and epoxy polyol resin, and combinations of resins of the same kind, of which molecular weight distributions are significantly different, or of which substituents are entirely different.

Any conventionally known dyes and pigments can be used as the coloring agents for use in the present invention. Examples of the dyes and pigments are carbon black, nigrosine dyes, black iron oxide, Naphthol Yellow S, Hansa Yellow (10G, 5G, G), cadmium yellow, yellow iron oxide, yellow ochre, chrome yellow pigment, Titan Yellow, Polyazo Yellow, oil Yellow, Hansa Yellow (GR, A, RN, R), Pigment Yellow L, Benzidine Yellow (G, GR), Permanent Yellow (NCG), Vulcan Fast Yellow (5G, R), Tartrazine Lake, Quinoline Yellow Lake, Anthragen Yellow BGL, isoindolinone yellow, red oxide, red lead, cadmium red, cadmium mercury red, antimony red, Permanent Red 4R, Para Red, Fire Red, p-chloro-o-nitroaniline red, Lithol Fast Scarlet G, Brilliant Fast Scarlet, Brilliant Carmine BS, Permanent Red (F2R, F4R, FRL, FRLL, F4RH), Fast Scarlet VD, Vulcan Fast Rubine B, Brilliant Scarlet G, Lithol Rubine GX, Permanent Red F5R, Brilliant Carmine 6B, Pigment Scarlet 3B, Bordeaux 5B, Toluidine Maroon, Permanent Bordeaux F2K, Helio Bordeaux BL, Bordeaux 10B, BON Maroon Light, BON Maroon Medium, eosine lake, Rhodamine Lake B, Rhodamine Lake Y, Alizarine Lake, Thioindigo Red B, Thioindigo Maroon, oil Red, quinacridone red, Pyrazolone Red, Polyazo Red, Chrome Vermilion, Benzidine Orange, Perynone Orange, Oil Orange, cobalt blue, cerulean blue, Alkali Blue Lake, Peacock Blue Lake, Victoria Blue Lake, metal-free phthalocyanine blue, Phthalocyanine Blue, Fast Sky Blue, Indanthrene Blue (RS, BC), indigo, ultramarine, Prussian blue, Anthraquinone Blue, Fast Violet B, Methyl Violet Lake, cobalt violet, manganese violet, dioxazine violet, Anthraquinone Violet, chrome green, zinc green, chrome oxide green, Persian, emerald green, Pigment Green B, Naphthol Green B, Green Gold, Acid Green Lake, Malachite Green Lake, Phthalocyanine Green, Anthraquinone Green, titanium oxide, zinc white, and lithopone. These dyes and pigments can be used in combination.

It is preferable that the amount of the coloring agent be in the range of 0.1 to 50 parts by weight to 100 parts by weight of the binder resin.

The toner of the present invention may further comprise a charge controlling agent. Any conventional charge controlling agents can be used in the toner of the present invention. For instance, a nigrosine dye, a triphenylmethano dye, a chromium-containing metal complex dye, a molybdic acid chelate pigment, a rhodamine dye, an alkoxyamine, a quaternary ammonium salt including a fluorine-modified quaternary ammonium salt, alkylamide, phosphorus and a phosphorus-containing compound, tungsten and a tungsten-containing compound, a fluorine-containing active material, and a metallic salt of salicylic acid and a metallic salt of a salicylic acid derivative are usable.

The amount of such charge controlling agent in the toner of the present invention depends upon the kind of the binder resin used in the toner and the use or non-use or an additive, and also upon the method of producing the toner, including the method of dispersing the necessary components for the toner. It is preferable that the amount of the charge controlling agent be in the range of 0.1 to 10 parts by weight, more preferably in the range of 2 to 5 parts by weight, to 100 parts by weight of the binder resin.

When the amount of the charge controlling agent is less than 0.1 parts by weight to 100 parts by weight of the binder resin, the negative chargeability of the toner tends to be insufficient for use in practice, while when the amount of the charge controlling agent is more than 10 parts by weight to 100 parts by weight of the binder resin, the negative chargeability of the toner tends to be excessively large so that the electrostatic attraction between a carrier or a charging member and the toner is excessively increased, or the fluidity of the toner is decreased, resulting in the lowering of image density.

Figure shows a schematic cross-sectional view of a one-component type development apparatus for use in the present invention.

In Figure, toner 7 held in a toner tank 1 is mixed and transported onto a toner bearing member 2 by a stirring blade 6 and a toner supply member 4. The toner 7 supplied onto the toner supply member 4 is made a thin layer of the toner 7 and is electrically charged by a toner layer thickness regulating member 3. The thus charged thin layer of the toner 7 is then transported into a development gap 8 between the surface of the toner bearing member 2 and a peripheral surface of a latent electrostatic image bearing member 5, so that latent electrostatic images formed on the surface of the latent electrostatic image bearing member 5 are developed with the toner 7 of the thin layer of the toner 7 to visible toner images (not shown). The toner images are then transferred to an intermediate image transfer member 9, whereby a first image transfer is carried out. The toner images transferred to the surface of the intermediate image transfer member 9 are then transferred to an image transfer material 11 by an image transfer roller 10, whereby a second image transfer is carried out. The toner images transferred to the image transfer material 11 are fixed thereto in an image fixing unit comprising a pair of image fixing rollers. Thus, fixed toner images are obtained on the image transfer material 11.

In the case of the development of full-color images, the development is carried out, successively using black, cyan, magenta and yellow toners and superimposing toner images developed with these color toners, whereby full-color images are obtained.

Other features of this invention will become apparent in the course of the following description of exemplary embodiments, which are given for illustration of the invention and are not intended to be limiting thereof.

### Example 1

### [Preparation of Black Toner No. 1]

A mixture or the following components with the following formulation was well mixed in a flusher:

To the above mixture, 1200 parts by weight of polyester resin (acid value: 3; hydroxyl value: 25; Mn: 45000; Mw/Mn: 4.0; Tg: 60°C) were added, and the mixture was kneaded at 150°C for 30 minutes.

To this kneaded mixture, 1000 parts by weight of xylene were added, and the mixture was kneaded for 1 hour. The water and the xylene were removed from the kneaded mixture, and the mixture was then subjected to roll-out cooling and pulverized, using a pulverizer, whereby a masterbatch pigment was obtained.

A mixture of the following components with the following formulation was mixed in a mixer:

The above mixture was fused and kneaded, using a two-roll mill. The kneaded mixture was then subjected to roll-out cooling, whereby a pigment composed of pigment particles with a maximum particle size of 0.4 µm was obtained. The pigment was then pulverized and classified, whereby a precursor toner composed of toner particles with a volume mean diameter of 7.5 µm was obtained. 0.8 parts by weight of a commercially available hydrophobic silica (Trademark "R972" made by Nippon Aerosil Co., Ltd.) were added to 100 parts by weight of the above precursor toner. This mixture was mixed in a mixer, whereby a black toner No. 1 of the present invention was obtained.

The aggregation degree of the black toner No. 1 was measured, using the above-mentioned commercially available powder tester (made by Hosokawa Micron Corporation), the 75 µm mesh sieve, the 45 µm mesh sieve, and the 22 µm mesh sieve, with 2 g of a sample of the black toner No. 1 placed in the uppermost 75 µm mesh sieve, with 30-second vibrations of the sieves. The result was that the aggregation degree of the black toner No. 1 was 10.2%.

### [Preparation of Yellow Toner No. 1]

A mixture of the following components with the following formulation was well mixed in a flusher:

To the above mixture, 1200 parts by weight of polyester resin (acid value: 3; hydroxyl value: 25; Mn: 45000; Mw/Mn: 4.0; Tg: 60°C) were added, and the mixture was kneaded at 150°C for 30 minutes.

To this kneaded mixture, 1000 parts by weight of xylene were added, and the mixture was kneaded for 1 hour. The water and the xylene were removed from the kneaded mixture, and the mixture was then subjected to roll-out cooling and pulverized, using a pulverizer. The pulverized mixture was then caused to pass through a 3-roll mill, with two passes, whereby a masterbatch pigment was obtained.

A mixture of the following components with the following formulation was mixed in a mixer:

The above mixture was fused and kneaded, using a two-roll mill. The kneaded mixture was then subjected to roll-out cooling, whereby a pigment composed of pigment particles with a maximum particle size of 0.4 µm was obtained. The pigment was then pulverized and classified, whereby a precursor toner composed of toner particles with a volume mean diameter of 7.5 µm was obtained. 0.8 parts by weight of a commercially available hydrophobic silica (Trademark "R972", made by Nippon Aerosil Co., Ltd.) were added to 100 parts by weight of the above precursor toner. This mixture was mixed in a mixer, whereby a yellow toner No. 1 of the present invention was obtained.

The aggregation degree of the yellow toner No. 1 was 11.5% when measured in the same manner as in the case of the black toner No. 1.

### [Preparation of Magenta Toner No. 1]

A mixture of the following components with the following formulation was well mixed in a flusher:

To the above mixture, 1200 parts by weight of polyester resin (acid value: 3; hydroxyl value: 25; Mn: 45000; Mw/Mn: 4.0; Tg: 60°C) were added, and the mixture was kneaded at 150°C for 30 minutes.

To this kneaded mixture, 1000 parts by weight of xylene were added, and the mixture was kneaded for 1 hour. The water and the xylene were removed from the kneaded mixture, and the mixture was then subjected to roll-out cooling and pulverized, using a pulverizer. The pulverized mixture was then caused to pass through a 3-roll mill, with two passes, whereby a masterbatch pigment was obtained.

A mixture of the following components with the following formulation was mixed in a mixer:

The above mixture was fused and kneaded, using a two-roll mill. The kneaded mixture was then subjected to roll-out cooling, whereby a pigment composed of pigment particles with a maximum particle size of 0.4 µm was obtained. The pigment was then pulverized and classified, whereby a precursor toner composed of toner particles with a volume mean diameter of 7.5 µm was obtained. 0.8 parts by weight of a commercially available hydrophobic silica (Trademark "R972", made by Nippon Aerosil Co., Ltd.) were added to 100 parts by weight of the above toner. This mixture was mixed in a mixer, whereby a magenta toner No. 1 of the present invention was obtained.

The aggregation degree of the magenta toner No. 1 was 10.5% when measured in the same manner as in the case of the black toner No. 1.

### [Preparation of Cyan Toner No. 1]

A mixture of the following components with the following formulation was well mixed in a flusher:

To the above mixture, 1200 parts by weight of polyester resin (acid value: 3; hydroxyl value: 25; Mn: 45000; Mw/Mn: 4.0; Tg: 60°C) were added, and the mixture was kneaded at 150°C for 30 minutes.

To this kneaded mixture, 1000 parts by weight of xylene were added, and the mixture was kneaded for 1 hour. The water and the xylene were removed from the kneaded mixture, and the mixture was then subjected to roll-out cooling and pulverized, using a pulverizer. The pulverized mixture was then caused to pass through a 3-roll mill, with two passes, whereby a masterbatch pigment was obtained.

A mixture of the following components with the following formulation was mixed in a mixer:

The above mixture was fused and kneaded, using a two-roll mill. The kneaded mixture was then subjected to roll-our cooling, whereby a pigment composed of pigment particles with a maximum particle size of 0.4 µm was obtained. The pigment was then pulverized and classified, whereby a precursor toner composed of toner particles with a volume mean diameter of 7.5 µm was obtained. 0.8 parts by weight of a commercially available hydrophobic silica (Trademark "R972", made by Nippon Aerosil Co., Ltd.) were added to 100 parts by weight of the above precursor toner. This mixture was mixed in a mixer, whereby a cyan toner No. 1 of the present invention was obtained.

The aggregation degree of the cyan toner No. 1 was 11.8% when measured in the same manner as in the case of the black toner No. 1.

By use of the above prepared black toner No. 1, yellow toner No. 1, magenta toner No. 1, and cyan toner No. 1, a full-color image was formed using the one-component development apparatus provided with the intermediate image transfer belt 9 for the first image transfer and the image transfer material for the second image transfer as shown in Figure. The thus obtained full-color image was compared with a limit sample and evaluated with respect to the formation of non-transferred spots, image thickening, the deposition of the toner on the background of the image, and the above-mentioned dull image formation, which means a potential problem that developed images are dull, unclear and, particularly unsharp in line images, and are not in the right positions as mentioned above.

The results are shown in TABLE 1.

### Example 2

The procedure of the preparation of each of black toner No. 1, yellow toner No. 1, magenta toner No. 1, and cyan toner No. 1 in Example 1 was repeated except that 0.8 parts by weight of a commercially available hydrophobic silica (Trademark "R972" made by Nippon Aerosil Co., Ltd.) added to 100 parts by weight of the precursor toner for each of the above toners were replaced with 1.0 part by weight of titanium oxide (Trademark "MT-150A", made by Tayca Co., Ltd.), whereby black toner No. 2, yellow toner No. 2, magenta toner No. 2, and clan toner No. 2 were prepared.

By use of the above prepared black toner No. 2, yellow toner No. 2, magenta toner No. 2, and cyan toner No. 2, a full-color image was formed using the same one-component development apparatus as used in Example 1, and evaluated in the same manner as in Example 1.

The results are shown in TABLE 1.

### Example 3

The procedure of the preparation of each of black toner No. 1, yellow toner No. 1, magenta toner No. 1, and cyan toner No. 1 in Example 1 was repeated except that 0.8 parts by weight of a commercially available hydrophobic silica (Trademark "R972" made by Nippon Aerosil Co., Ltd.) added to 100 parts by weight of the precursor toner for each of the above toners were replaced with a mixture of 0.6 parts by weight of hydrophobic silica (Trademark "H2000" made by Hoechst Japan Ltd.) and 0.9 parts of titanium oxide (Trademark "MT-150A", made by Tayca Co., Ltd.), whereby black toner No. 3, yellow toner No. 3, magenta toner No. 3, and cyan toner No. 3 were prepared.

By use of the above prepared black toner No. 3, yellow toner No. 3, magenta toner No. 3, and cyan toner No. 3, a full-color image was formed using the same one-component development apparatus as used in Example 1, and evaluated in the same manner as in Example 1.

The results are shown in TABLE 1.

### Example 4

The procedure of the preparation of each of black toner No. 1, yellow toner No. 1, magenta toner No. 1, and cyan toner No. 1 in Example 1 was repeated except that the polyester resin (acid value: 3; hydroxyl value: 25; Mn: 45000; Mw/Mn: 4.0; Tg: 60°C) was replaced by epoxy polyol resin (Mn: 3800; Mw/Mn: 3.9; Tg: 59°C) and that 0.8 parts by weight of a commercially available hydrophobic silica (Trademark "R972" made by Nippon Aerosil Co., Ltd.) added to 100 parts by weight of the precursor toner for each of the above toners were replaced with a mixture of 0.6 parts by weight of hydrophobic silica (Trademark "H2000" made by Hoechst Japan Ltd.) and 0.9 parts of titanium oxide (Trademark "MT-150A", made by Tayca Co., Ltd.), whereby black toner No. 4, yellow toner No. 4, magenta toner No. 4, and cyan toner No. 4 were prepared.

By use of the above prepared black toner No. 4, yellow toner No. 4, magenta toner No. 4, and cyan toner No. 4, a full-color image was formed using the same one-component development apparatus as used in Example 1, and evaluated in the same manner as in Example 1.

The results are shown in TABLE 1.

### Example 5

The procedure of the preparation of each of black toner No. 4, yellow toner No. 4, magenta toner No. 4, and cyan toner No. 4 in Example 4 was repeated except that the precursor toner for each of the above toners was stirred for 300 seconds and the mixture of 0.6 parts by weight of hydrophobic silica (Trademark "H2000" made by Hoechst Japan Ltd.) and 0.9 parts of titanium oxide (Trademark "MT-150A", made by Tayca Co., Ltd.) was added within 2 minutes after the completion of the stirring of the precursor toner for 300 seconds, whereby black toner No. 5, yellow toner No. 5, magenta toner No. 5, and clan toner No. 5 were prepared.

By use of the above prepared black toner No. 5, yellow toner No. 5, magenta toner No. 5, and cyan toner No. 5, a full-color image was formed using the same one-component development apparatus as used in Example 1, and evaluated in the same manner as in Example 1.

The results are shown in TABLE 1.

### Comparative Example 1

The procedure of the preparation of each of black toner No. 1, yellow toner No. 1, magenta toner No. 1, and cyan toner No. 1 in Example 1 was repeated except that the precursor toner was subjected to heat treatment by the toner particles thereof being exposed to hot air, thereby making the toner particles spherical, and that 0.8 parts by weight of a commercially available hydrophobic silica (Trademark "R972" made by Nippon Aerosil Co., Ltd.) added to 100 parts by weight of the precursor toner for each of the above toners ere replaced with 0.8 parts by weight of hydrophobic silica (Trademark "H2000" made by Hoechst Japan Ltd.), whereby comparative black toner No. 1, comparative yellow toner No. 1, comparative magenta toner No. 1, and comparative cyan toner No. 1 were prepared.

By use of the above prepared comparative black toner No. 1, comparative yellow toner No. 1, comparative magenta toner No. 1, and comparative cyan toner No. 1, a full-color image was formed using he same one-component development apparatus as used in Example 1, and evaluated in the same manner as in Example 1.

The results are shown in TABLE 1.

### Comparative Example 2

The procedure of the preparation of each of black toner No. 1, yellow toner No. 1, magenta toner No. 1, and cyan toner No. 1 in Example 1 was repeated except that 0.8 parts by weight of a commercially available hydrophobic silica (Trademark "R972" made by Nippon Aerosil Co., Ltd.) added to 100 parts by weight of the precursor toner for each of the above toners were replaced with 1.2 Parts by weight of hydrophobic silica (Trademark "H2000" made by Hoechst Japan Ltd.), whereby comparative black toner No. 2, comparative yellow toner No. 2, comparative magenta toner No. 2, and comparative cyan toner No. 2 were prepared.

By use of the above prepared comparative black toner No. 2, comparative yellow toner No. 2, comparative magenta toner No. 2, and comparative cyan toner No. 2, a full-color image was formed using the same one-component development apparatus as used in Example 1, and evaluated in the same manner as in Example 1.

The results are shown in TABLE 1.

### Comparative Example 3

The procedure of the preparation of each of black toner No. 1, yellow toner No. 1, magenta toner No. 1, and cyan toner No. 1 in Example 1 was repeated except that 0.8 parts by weight of a commercially available hydrophobic silica (Trademark "R972" made by Nippon Aerosil Co., Ltd.) added to 100 parts by weight of the precursor toner for each of the above toners were replaced with 0.05 parts by weight of hydrophobic silica (Trademark "H2000" made by Hoechst Japan Ltd.), whereby comparative black toner No. 3, comparative yellow toner No. 3, comparative magenta toner No. 3, and comparative cyan toner No. 3 were prepared.

By use of the above prepared comparative black toner No. 3, comparative yellow toner No. 3, comparative magenta toner No. 3, and comparative cyan toner No. 3, a full-color image was formed using the same one-component development apparatus as used in Example 1, and evaluated in the same manner as in Example 1.

The results are shown in TABLE 1.

In the above TABLE 1, a maximum aggregation degree and a minimum aggregation degree are provided, which are determined from four aggregation degrees obtained by measuring the aggregation degree of each of the four color toners in each Example.

With respect to the evaluation ranks, "5" denotes "excellent", free of the problem, "3" denotes "acceptable for use in practice", despite the problem, and "1" denotes "no good", due to the problem, and "4" is between the rank "5" and the rank "3", and "2" is between the rank "1" and the rank "3" by visual inspection of the developed toner images.

All of the tested toner particles had an average particle size in a range of 5 to 10 µm.

## Claims

1. A toner for developing latent electrostatic images to toner images for use in an intermediate transfer image formation method comprising the steps of forming a thin layer of toner on a toner bearing member, triboelectrically charging the toner to a predetermined polarity using a triboelectric charging member, developing latent electrostatic images formed on an image bearing member to toner images with said toner, transferring said developed toner images to an intermediate image transfer member which runs along an endless path, thereby subjecting said developed toner images to a first image transfer, and transferring said toner images transferred to said intermediate image transfer member to an image transfer material, thereby subjecting said developed toner images to a second image transfer, comprising:
toner particles comprising a coloring agent and a binder resin, with an average particle size in a range of 5 to 10 µm and an aggregation degree of 5 to 20%.

2. The toner as claimed in Claim 1, further comprising finely-divided particles of silica which are made hydrophobic in an amount ratio of 0.1 to 1.0 parts by weight to 100 parts by weight of said toner.

3. The toner as claimed in Claim 1, further comprising finely-divided particles of titanium oxide in an amount ratio of 0.1 to 1.2 parts by weight to 100 parts by weight of said toner.

4. The toner as claimed in Claim 1, further comprising (a) finely-divided particles of silica which are made hydrophobic and (b) finely-divided particles of titanium oxide in a parts-by-weight ratio of 1 : 9 to 6 : 4.

5. The toner as claimed in any one of Claims 1-4, wherein said binder resin is a polyol resin.

6. A method of producing a toner comprising toner particles comprising a coloring agent and a binder resin, and at least one additive component, comprising the steps of:
stirring said toner particles alone, and then
mixing said toner particles with said additive component.

7. The method as claimed in Claim 6, wherein said additive component is selected from the group consisting of (a) finely-divided particles of silica which are made hydrophobic and (b) finely-divided particles of titanium oxide.

8. An intermediate transfer image formation method comprising the steps of:
forming a thin layer of toner on a toner bearing member, triboelectrically charging the toner to a predetermined polarity using a triboelectric charging member, developing latent electrostatic images formed on an image bearing member to toner images with said toner, transferring said developed toner images to an intermediate image transfer member which runs along an endless path, thereby subjecting said developed toner images to a first image transfer, and transferring said toner images transferred to said intermediate image transfer member to an image transfer material, thereby subjecting said developed toner images to a second image transfer, wherein as said toner is used a toner which comprises toner particles comprising a coloring agent and a binder resin, with an average particle size in a range of 5 to 10 µm and an aggregation degree of 5 to 20%.

9. The intermediate transfer image formation method as claimed in Claim 8, wherein said toner further comprises finely-divided particles of silica which are made hydrophobic in an amount ratio of 0.1 to 1.0 parts by weight to 100 parts by weight of said toner.

10. The intermediate transfer image formation method as claimed in Claim 8, wherein said toner further comprises finely-divided particles of titanium oxide in an amount ratio of 0.1 to 1.2 parts by weight to 100 parts by weight of said toner.

11. The intermediate transfer image formation method as claimed in Claim 8, wherein said toner further comprises (a) finely-divided particles of silica which are made hydrophobic and (b) finely-divided particles of titanium oxide in a parts-by-weight ratio of 1 : 9 to 6 : 4.

12. The intermediate transfer image formation method as claimed in any one of Claims 8-11, wherein said binder resin is a polyol resin.
